

Patented Aug. 16, 1927.

1,639,347

# UNITED STATES PATENT OFFICE.

LUTHER B. LOCKHART, OF ATLANTA, GEORGIA, ASSIGNOR TO STANDARD OIL COMPANY, OF WHITING, INDIANA, A CORPORATION OF INDIANA.

## LUBRICANT FOR AUTOMOTIVE ENGINES.

No Drawing.

Application filed February 20, 1926. Serial No. 89,764.

This invention relates to a composition of matter for use in lubricating internal combustion engines, particularly of the type employed in automotive vehicles employing 5 gasoline as a fuel and in which constituents of the fuel enter the lubricant in the crank-case. It is particularly adapted for use in cold weather, facilitating starting and lubrication of the bearings of the motor when 10 fresh and suffering little or practically no loss or viscosity by dilution in an average car in ordinary winter operation with proper carburetor adjustment.

The lubricant oil of my invention is clear 15 in appearance, and free from suspended solids, colloidal carbon and marked disagreeable odor. It has a viscosity of not less than 140 seconds Saybolt at 100° F., a flash point in excess of 110° F., and preferably 20 above 150° F., and on distillation yields from 5 to 15% (and preferably from 7 to 15%) of fractions boiling above 300° F. and below 460° F. Such an oil adequately lubricates the bearings of the motor while 25 cold, and shows very little if any loss in viscosity during use, and particularly during the first 100 miles of operation, thereby differing markedly from oils previously known. A preferred oil in accordance with 30 this invention is one having a viscosity of about 184 seconds Saybolt at 100° F. a flash point of about 150° F., and containing about 8% of fractions boiling between 320° and 450° F., the remainder having a viscosity 35 of 340 to 350.

Such an oil may be produced by an admixing with 92 parts of a viscous lubricant oil, for example, of paraffin type or a mid-continent oil, having a viscosity of 340 to 40 350 sec. Saybolt at 100° F. about 8 parts of a light distillate oil having a boiling point range of 320° to 460° F.

It is, of course, apparent that the composition of the oil may be varied within wide

limits and still retain the principles of the 45 invention embodied herein. The specific details above set forth are not intended to be regarded as limitations upon the scope of the invention, except in so far as included in the accompanying claims. 50

### I claim:

1. The herein described marketable lubricating oil for cold weather use in automotive engines of the type in which liquid fuel enters the oil from the cylinders, clear in 55 appearance, free from suspended solids, colloidal carbon and marked disagreeable odor, and characterized further by having a flash point above 150° F., a Saybolt viscosity of at least 140 at 100° F., a relatively low loss 60 in viscosity during use and a content of between 7 and 15% of fractions boiling between about 300° F. and 460° F.

2. The herein described marketable lubricating oil for cold weather use in automotive engines of the type in which liquid fuel enters the oil from the cylinders, clear in 65 appearance, free from suspended solids, colloidal carbon and marked disagreeable odor, said oil having a viscosity of about 70 184 seconds Saybolt at 100° F., and on distillation showing a content of about 8% of fractions boiling between 300° F. and 450° F.

3. The herein described marketable lubricating oil for cold weather use in automotive engines of the type in which liquid fuel enters the oil from the cylinders, clear in 75 appearance, free from suspended solids, colloidal carbon and marked disagreeable 80 odor, and characterized further by having a flash point above 150° F., a Saybolt viscosity of at least 140 at 100° F., a relatively low loss 85 in viscosity during use and a content of between 5 and 15% of fractions boiling between about 300° F. and 460° F.

LUTHER B. LOCKHART